

## UNITED STATES PATENT OFFICE

2,266,952

STAINLESS STEEL TREATMENT AND  
PRODUCT

Fredrick Kenneth Bloom, Baltimore, Md., assignor to Rustless Iron and Steel Corporation, Baltimore, Md., a corporation of Delaware

No Drawing. Application December 26, 1939,  
Serial No. 311,014

5 Claims. (Cl. 148—12)

My invention relates to a process for treating stainless steel products, and more particularly to the treating of those products which can be hardened by heat treatment.

One of the objects of my invention is to provide a simple, practical and efficient method of producing stainless steel products to achieve a desired high elastic limit in combination with high ultimate strength and hardness.

Another object is to provide a process whereby hardenable stainless steel products may be given a high elastic limit in a direct and reliable manner without sacrifice to ductility.

A further object of my invention is to produce stainless steel products, such as rods and wire of high elastic limit, and to provide a simple method of achieving the same, which subsequently may be fabricated into articles of ultimate use without substantial loss of this property.

Other objects in part will be obvious and in part will be pointed out hereinafter.

The invention accordingly consists in the combination of steps and the relation of each of the same to one or more of the others as described herein, and in the resultant products or articles therefrom, the scope of the application of which is indicated in the following claims.

As conducive to a clearer understanding of certain features of my invention, it may be noted at this point that there are many applications in which it is desirable to have a corrosion resistant metal which is hard and also has the property of high elasticity. A high elastic limit is essential where the material must be able to bend under an appreciable stress without taking a permanent set, and must return to its original shape after the stress is removed. Examples of applications in which such properties are needed are automobile steering wheel spokes, pole type radio aerials, and the like.

Desired corrosion resistance in combination with strength and hardness is achieved to a fair degree in the hardenable stainless steels. These have a carbon content of about 0.08% to 0.50% and a chromium content of about 12% to 17%, with or without a nickel content of some 1.5 or 2%. Other ingredients, such as copper and molybdenum in small amounts, also may be present.

Heretofore, it has been the practice to harden such steels by heating them to 1750° to 1950° F., which is within their range of solid solution and then quenching. This operation gives a satisfactory hardness but for certain applications the resulting elastic limit is undesirably low.

Where hardening treatment is followed by a tempering or strain relieving process, it is found that the elastic property of the steel is considerably improved. This tempering process consists of heating the metal to some temperature between 400° and 1100° F. and cooling. This operation follows the hardening treatment. The lowest possible tempering temperature is used in obtaining the mechanical properties desired, preferably not above 930° F., since it is found that the lower temperatures have less deleterious effect on corrosion resistance.

The elastic limit obtained by the above-mentioned hardening and tempering operations still is not as high as is desirable for applications where the metal must be able to withstand a high stress without suffering a permanent set. Accordingly, one of the objects of my invention is the provision of a simple, efficient and practical method of achieving, in the stainless steels of the hardenable types, a higher elastic limit than heretofore has been obtained, in combination with high strength and hardness and without substantial loss in ductility.

Referring now more particularly to the practice of my invention, I find that excellent elastic properties of stainless steels are obtained by a particular combination of working and heating treatments. I find that by slightly cold working the metal after a hardening operation and following this by a treatment of tempering, exceptional results are had. Only a small amount of cold work is necessary. Good results are had both where the cold work is by cold drawing and where it is by the alternate bending action of a straightening operation.

Hardenable stainless steels ordinarily are worked to a desired shape and size at the mill and hardened by quenching from a temperature above the carbide solution temperature before shipment. According to a standard mill practice, this working is conducted at a temperature, which usually is from about 1750° to 2050° F. In the practice of my invention, the greatest part of all of the reduction through rolling, drawing, etc., as usual may be done at this high temperature. The worked products conveniently are quenched from this working temperature to give a desired hardness. This hardening treatment is the first step in my process of obtaining stainless steel products of high elastic limit.

As a second step, the products then are given either a further reduction, as by bringing the products to size or desired finish, or they are straightened in such manner as to be subjected

to an alternate bending operation. I find that good results are obtained with either of these cold-working operations. In wire products, for example, a light reduction by cold drawing is eminently satisfactory. Excellent results likewise are had with only the mild form of cold working had in the alternate bending operation.

In connection with the second step of my process, it is to be noted that the cold working can be readily done on existing mill equipment without incurring any expense other than that involved in the ordinary rolling, drawing, straightening and other processes. Extra working equipment therefore is unnecessary to the practice of my invention. This, of course, is particularly important commercially since it permits the practice of the process without additional working costs.

After cold working the metal, I carry out the tempering treatment, representing the third step in my process. This consists in heating the metal to a temperature between 400° and 1100° F., preferably above 600° F. but below 930° F., for about one hour. I find that the major portion of the increase in elastic limit is had in the first ten minutes of tempering so that in many cases a desired increase in elastic limit is had where the tempering period is but some ten minutes in duration. The short tempering treatment has the special advantage of precluding any discoloration of the metal surface during tempering. Following the tempering treatment, the products are brought to room temperature for packing and shipping or storing, as desired.

To appreciate the advantages of my process, reference may be had to the following table, in which there are presented the physical properties of three different types of stainless steel in wire form which have been subjected to different treatments.

what increased over that resulting from the old practices.

While it is known that the physical properties of stainless steel, such as its ultimate strength, elastic limit and hardness, are improved through a hardening treatment or through a cold-working operation, these all usually increase in substantially like amounts. In the cold-working step of my invention, therefore, it reasonably might be expected that a slight improvement in the physical properties would result. I find, however, as pointed out above, that where this cold-working step is combined with a preceding hardening treatment and a succeeding tempering treatment, there is a phenomenal increase in but one of these properties, namely the elastic limit. The others appear to be affected only as might be expected. Although I am unable to account for this surprising phenomenon, it is an observed fact as shown above. This unexpected property of my process gives products such as rods and wire which are particularly adapted to applications where elasticity in combination with one or more of strength, ductility and corrosion resistance, is important. Among these applications are automobile steering wheel spokes and automobile radio antennas. Also, both in wire and strip form, the material is useful in all manner of springs and supports where elasticity is required.

Thus it will be seen that there is provided in my invention a method of treating stainless steel products to achieve a desired high elastic limit in combination with strength, ductility and corrosion resistance, wherein the objects hereinbefore noted, together with many thoroughly practical advantages are successfully achieved. Moreover, the process of my invention can readily be carried out with equipment already present in

| Analysis of stainless steel  | Processing method |                                        | Ultimate tensile strength    | Elastic limit               | Elongation in 2 in. | Rockwell hardness |
|------------------------------|-------------------|----------------------------------------|------------------------------|-----------------------------|---------------------|-------------------|
|                              | Type              | Procedure                              |                              |                             |                     |                   |
| C 0.11%; Cr 12.55%           | Old treatment     | Hardened only                          | Lbs. per. sq. in.<br>196,000 | Lbs. per. sq. in.<br>73,000 | Per cent<br>7.0     | C 41              |
|                              | do                | Hardened and tempered.                 | 193,000                      | 106,000                     | 7.0                 | C 41              |
|                              | New treatment     | Hardened, cold-drawn 15% and tempered. | 198,000                      | 180,000                     | 7.0                 | C 41              |
|                              | do                | Hardened, straightened and tempered.   | 206,000                      | 188,000                     | 7.5                 | C 42              |
|                              | Old treatment     | Hardened and tempered.                 | 218,000                      | 130,000                     | 6.5                 | -----             |
|                              | New treatment     | Hardened, cold-drawn 5% and tempered.  | 230,000                      | 220,000                     | 5.5                 | -----             |
| C 0.38%; Cr 13.49%           | Old treatment     | Hardened only                          | 217,000                      | 79,000                      | 8.0                 | C 45              |
|                              | do                | Hardened and tempered.                 | 219,500                      | 130,000                     | 8.0                 | C 44              |
| C 0.13%; Cr 14.70%; Ni 2.05% | New treatment     | Hardened, straightened and tempered.   | 232,000                      | 218,000                     | 6.0                 | C 45              |

From an inspection of the table given above, it will be seen that steel which has been subjected to my improved process suffers no decrease in hardness and very little, if any, decrease in ductility. The elastic limit of the metal is materially greater than that resulting from the standard processes of hardening or hardening and tempering. I find that the elastic limits of the stainless steel products of my invention amount to some 250% of those of like products which merely are hardened by heat treatment. As compared to stainless steel products which have been hardened and tempered, I find that my products have elastic limits amounting to some 160% to 180% of those products. Furthermore, by my process the tensile strength is some-

60 mills and in a simple manner entailing a minimum of additional expense.

As many possible embodiments may be made of my invention, and as many changes may be made in the embodiment herein set forth, it will be understood that all matter described herein is to be interpreted as being illustrative and not as being a limitation.

I claim:

70 1. In treating stainless steel products which are hardened by heat treatment and contain 12 per cent to 17 per cent chromium and .08 per cent to .50 per cent carbon, the art which comprises, quenching said products from a temperature between 1750° F. and 1950° F., cold-working the same to an extent between a light finishing reduc-

tion to size and a reduction of 15 per cent, and then tempering said products at a temperature of from 400° F. to 1100° F.

2. In treating stainless steel products which are hardenable by heat treatment and contain 12 per cent to 17 per cent chromium and .08 per cent to .50 per cent carbon, the art which comprises, first hardening said products, then giving the same a cold reduction of about 5 per cent, and then tempering the same at about 930° F.

3. In treating stainless steel wire which is hardenable by heat treatment and contain 12 per cent to 17 per cent chromium and .08 per cent to .50 per cent carbon, the art which comprises, quenching the wire from a temperature of 1750° to 1950° F., then subjecting the wire to a cold-working operation as by the alternate bending of a straightening operation or a light cold-drawing which should not exceed a reduction of 15 per

cent, and thereafter heating the wire to a temperature of 400° F. to 1100° F., and subsequently cooling the same to room temperature.

4. In treating stainless steels which are hardenable by heat treatment having a content of 0.08 per cent to 0.50 per cent carbon, 12 per cent to 17 per cent chromium, the art which comprises, hardening the metal, cold working the same by a light finishing operation, and then tempering the metal at a temperature between 600° F. and 930° F.

5. In manufactures of the class described, hardened stainless steel wire including about .08 per cent to .50 per cent carbon and 12 per cent to 17 per cent chromium, subjected to the cold work of a straightening operation and tempered to achieve high elastic strength in combination with desired hardness and ductility.

FREDRICK KENNETH BLOOM.